# EUROPEAN PATENT SPECIFICATION

(11) **EP 0 497 410 B1**
(45) Date of publication and mention of the grant of the patent: **27.03.1996**
(21) Application number: 92200179.7
(22) Date of filing: 23.01.1992
(51) Int. Cl.: C25C 3/00, C25C 3/24

(54) **Method for altering the concentration of a chemical element in liquid metal via an electrochemical way**
Verfahren zur Änderung der Konzentration eines chemischen Elementes in einem flüssigen Metall auf elektrochemischem Wege
Méthode pour modifier la concentration d'un élément chimique dans un métal liquide par voie électrochimique

(30) Priority: 29.01.1991 BE 9100080
(43) Date of publication of application: 05.08.1992
(73) Proprietor: "VLAAMSE INSTELLING VOOR TECHNOLOGISCH ONDERZOEK", afgekort "V.I.T.O.", B-2400 Mol (BE)
(72) Inventor: Dekeyser, Jacky C., B-3910 Neerpelt (BE); de Schutter, François J.E., B-2440 Geel (BE); Leysen, Roger F.R., B-2400 Mol (BE)
(74) Representative: Debrabandere, René

(56) References cited:
- EP-A- 0 267 054
- US-A- 3 980 499
- US-A- 4 203 819
- US-A- 4 882 017
- PATENT ABSTRACTS OF JAPAN vol. 4, no. 16 (C-072)7 February 1980 & JP-A-54 152 611 (KOLBE STEEL LTD) 1 December 1979

## Description

The present invention concerns a method for altering the concentration of at least lithium in a liquid metal of the group composed of aluminium, copper, zinc, tin and lead comprising lithium and at least one other chemical element of the group Ia of the periodic table of the elements, in an electrochemical way, according to which an electrochemical cell is formed with a solid electrolyte, having at one side the liquid metal and at the other side an electricity-conducting material wherein lithium can be absorbed, and whereby a DC voltage is produced between said electricity-conducting material and the liquid metal.

A frequent impurity in primary aluminium is sodium, which is found in the electrolytic bath (cryolite) during the production of aluminium (Hall-Héroult cycle). Lithium is also added to the bath during this process, such that this is also present as an impurity. Lithium is also a major impurity in secondary (recycled) aluminium, since for the making of aluminium use is often made of scrap metal from the airplane industry. In the future, said scrap metal will contain more and more lithium-aluminium alloys.

Until now, for various practical reasons, scrap metal from the airplane industry must be separated from other scrap metal as long as there is no adequate method to purify the aluminium from lithium.

Alkali metals such as lithium and sodium which are present in the liquid metal encourage crack formation during the rolling of the ingots.

The purification of the liquid metal can take place at a separate purification stage with chemical additives. It is also known, however, that said purification can be done in an electrochemical way. Such a purification method is described in patent US-A-4.849.072. According to this method lithium is removed from a melted lithium-aluminium alloy by means of an electrochemical cell having a melted, lithium-containing salt as an electrolyte, with the melted lithium-aluminium alloy at one side and melted lithium at the other side.

The altering of the lithium concentration in a liquid alloy of lithium and another metal, such as tin or aluminium, by means of an electrochemical cell with a solid electrolyte is described by H. Tuller and P. Moon in "Materials Science and Engineering", (Elsevier Sequoia), volume B1, (1988), page 189. According to this method, lithium can be extracted from an aluminium alloy so as to purify it. However, no other elements but lithium can be extracted from it such as for example sodium and potassium, since the solid electrolyte used only conducts lithium ions. For a lithium borate such as LiBO₂ is used as an electrolyte.

The present invention aims to correct these disadvantages and to provide a method for altering the concentration of a chemical element via an electrochemical way according to which an electrochemical cell with a solid electrolyte is formed, but whereby not only lithium but also other chemical elements of the group Ia of the periodic table of the elements can be extracted all at once from a metal, in particular aluminium, or can be put in such a bath.

To this aim, an electrochemical cell is formed with a solid electrolyte from a material conducting at the same time ions of lithium and ions of another element of the group Ia, said cell having at one side of the electrolyte the liquid metal and at the other side an electricity-conducting material in which the lithium and the other chemical element can be absorbed, and in that such DC voltage is produced between said electricity-conducting material and the liquid metal that the lithium and said other chemical element migrates at the same time through the solid electrolyte.

A method for removing sodium from molten aluminium in an electrochemical way is disclosed in Patent Abstracts of Japan, vol.4, no.16 (C-072) 07.02.1980 & JP-A-54.152.611. An electrochemical cell is used in which the molten metal forms the anode, the cathode being a metal having a melting point close to that of aluminium. The electrodes are separated by a beta-alumina solid electrolyte. Only sodium is removed from the liquid metal.

According to the invention, use is preferably made of a solid electrolyte from the beta-alumina family or from a sodium super ionic conductor based on sodium, zirconium and phosphate.

The use of a beta-alumina solid electrolyte is also mentioned in the above-mentioned publication and JP-A-54.152.611, but only for the electrolysis of melted sodium salts or for removing sodium from molten aluminium. The use of said electrolyte is obvious here, since it is known to be a good sodium ion conductor.

The applicant uses a sodium ion conductor having a mixed ion conductivity (e.g. sodium-beta-alumina). Although this material is a sodium conductor, the mobile sodium ions can nevertheless be replaced through interchange by other ions such as H₃O⁺, K⁺, Sr⁺, Li⁺, such that it can also be used to pump through other than Na⁺ ions. In particular, use is made of beta-alumina as a solid electrolyte, which is a mixed oxide composed of Al₂O₃ and Na₂O.

The working method described above is particularly interesting for altering the amount of lithium in liquid aluminium and in particular for purifying aluminium which has been polluted by lithium.

In the latter case, not only lithium is extracted from the aluminium-lithium alloy, but also other alkali metals or impurities.

It is advantageous to use bismuth or a bismuth alloy as a conductor.

Other particularities and advantages of the invention will become clear from the following description of a method for altering the concentration of at least lithium in a liquid metal via an electrochemical way according to the invention. This description is given as an example only and is not limitative in any way. The figures refer to the accompanying drawing which shows a cross section of a device for the application of the method according to the invention.

To purify melted aluminium which has been polluted by lithium, alkali metals or any other metallurgic impurities, an electrochemical cell is formed with said melted aluminium, a conductor and a solid electrolyte between the two of them, and a DC voltage is produced between the liquid metal and said conductor.

Use is made of a beta-alumina or beta"-alumina as a solid electrolyte, a mixed oxide composed of Al₂O₃ and Na₂O. Use can also be made of a "sodium super ionic conductor" (NASICON), which is a material based on sodium, zirconium and phosphate. Bismuth can be used as a conductor.

In order to bring lithium ions from the liquid aluminium bath in the bismuth, the liquid aluminium must be connected to the positive pole of a DC source and the bismuth with the negative pole of this source.

By sending a constant current through the solid electrolyte, the concentration of the positively charged ions will drop in the aluminium and increase in the bismuth.

The amount of material that is pumped through the solid electrolyte is determined by Faraday's law. For 26.8 Ah, one mole of monovalent, equivalent, ionized metal is pumped through the solid electrolyte. How the cell can be constructed in practice becomes clear from the accompanying drawing in which three cells are set up in parallel.

The liquid aluminium 1 is situated in the gutter 2. The aluminium 1 is present in all three cells at once. Each cell contains a tube 3 of sodium-beta-alumina closed off at the bottom which is filled with liquid bismuth 4.

The bismuth 4 in the three tubes is connected to the negative pole of a common DC-source 6 via conductors 5. The three amounts of bismuth are connected in parallel whereby the current is measured in the part of the conductors 5 which is connected to the bismuth in one tube 3, for example by measuring the tension by means of a voltmeter 7 over a rheostat 8 of one Ohm, which is connected in series to the cell.

The positive pole of the common power source 6 makes an electric contact with the aluminium 1 via the conductor 9 which is immersed in said aluminium. The following reaction takes place in the aluminium 1: M → M⁺ + e⁻, whereas in the bismuth 4 the following reaction takes place: M⁺ + e⁻ → M, whereby M can be hydrogen, sodium, lithium, etc.

Thus at the transition aluminium/beta-alumina, an electrochemical oxidation of lithium, sodium, hydrogen, etc. takes place. The thus formed ions migrate through the solid electrolyte, i.e. the tube 3 of sodium-beta-alumina, and are reduced at the transition beta-alumina/bismuth. The more cells are formed with the liquid aluminium, the greater the total current and thus the greater the purification capacity. In practice use will always be made of a battery of cells.

With a device as shown in the accompanying drawing and with pure bismuth in the sodium-beta-aluminium tubes 3, it was possible to remove a total mass of lithium, sodium and such like to the amount of 0.0384 g from the liquid aluminium with a total conducted charge of 0.1612 Ah.

The present invention is in no way limited to the embodiments described above.

## Claims

1. Method for altering the concentration of at least lithium in a liquid metal of the group composed of aluminium, copper, zinc, tin and lead, comprising lithium and at least one other chemical element of the group Ia of the periodic table of the elements, in an electrochemical way, according to which an electrochemical cell is formed with a solid electrolyte, having on one side the liquid metal and at the other side an electricity-conducting material wherein lithium can be absorbed, and whereby a DC voltage is produced between said electricity conducting material and the liquid metal, characterized in that the solid electrolyte is made from a material conducting at the same time ions of lithium and ions of another element of the group Ia, in that the electricity-conducting material is selected for absorbing the lithium and the other chemical element, and in that such DC voltage is produced between said electricity-conducting material and the liquid metal that the lithium and said other chemical element migrates at the same time through the solid electrolyte.

2. Method according to claim 1, characterized in that a solid electrolyte from the beta-alumina family is used.

3. Method according to claim 1, characterized in that a sodium super ionic conductor based on sodium, zirconium and phosphate is used as solid electrolyte.

4. Method according to any one of the preceding claims, characterized in that aluminium is used as liquid metal.

5. Method according to claim 4, characterized in that sodium is the other chemical element of the group Ia.

6. Method according to any one of the preceding claims, characterized in that bismuth or a bismuth alloy is used as electricity-conducting material.

## Patentansprüche

1. Verfahren zur Änderung der Konzentration von zumindest Lithium in einem flüssigen Metall der Gruppe, die sich aus Aluminium, Kupfer, Zink, Zinn und Blei zusammensetzt, welches Lithium und zumindest ein anderes chemisches Element der Gruppe Ia des Periodensystems der Elemente enthält, auf elektrochemischem Wege, gemäß welchen Verfahrens eine elektrochemische Zelle mit einem Trockenelektrolyten gebildet wird, die an einer Seite das flüssige Metall und an der anderen Seite ein elektrisch leitendes Material hat, worin Lithium absorbiert werden kann, und wobei eine Gleichspannung zwischen besagtem elektrisch leitendem Material und dem flüssigen Metall erzeugt wird, dadurch gekennzeichnet, daß der Trockenelektrolyt aus einem Material hergestellt ist, das gleichzeitig Lithiumionen und Ionen eines anderen Elements der Gruppe Ia leitet, dadurch, daß das elektrisch leitende Material zum Absorbieren des Lithiums und des anderen chemischen Elements gewählt ist, und dadurch, daß eine solche Gleichspannung zwischen besagtem elektrisch leitendem Material und dem flüssigen Metall erzeugt wird, daß das Lithium und besagtes anderes chemisches Element gleichzeitig durch den Trockenelektrolyten wandern.

2. Verfahren gemäß Anspruch 1, dadurch gekennzeichnet, daß ein Trockenelektrolyt aus der Beta-Aluminiumoxidfamilie verwendet wird.

3. Verfahren gemäß Anspruch 1, dadurch gekennzeichnet, daß ein Natrium-Superionenleiter auf Basis von Natrium, Zirkonium und einem Phosphat als Trockenelektrolyt verwendet wird.

4. Verfahren gemäß einem der vorgenannten Ansprüche, dadurch gekennzeichnet, daß Aluminium als flüssiges Metall verwendet wird.

5. Verfahren gemäß Anspruch 4, dadurch gekennzeichnet, daß Natrium das andere chemische Element aus der Gruppe Ia ist.

6. Verfahren gemäß einem der vorgenannten Ansprüche, dadurch gekennzeichnet, daß Wismut oder eine Wismutlegierung als elektrisch leitendes Material verwendet wird.

## Revendications

1. Procédé pour modifier la concentration au moins du lithium dans un métal liquide du groupe composé d'aluminium, de cuivre, de zinc, d'étain et de plomb, comprenant du lithium et au moins un autre élément chimique du groupe Ia du tableau périodique des éléments, d'une manière électrochimique, conformément auquel on forme une cellule électrochimique avec un électrolyte solide comportant, d'un côté, le métal liquide et, de l'autre côté, une matière électroconductrice dans laquelle du lithium peut être absorbé, et par lequel on génère une tension en courant continu entre ladite matière électroconductrice et le métal liquide, caractérisé en ce que l'électrolyte solide est réalisé à partir d'une matière qui conduit en même temps des ions de lithium et des ions d'un autre élément du groupe Ia, en ce que la matière électroconductrice est choisie pour absorber le lithium et l'autre élément chimique, et en ce qu'on génère une tension de courant continu entre ladite matière électroconductrice et le métal liquide, telle que le lithium et ledit autre élément chimique migrent en même temps à travers l'électrolyte solide.

2. Procédé selon la revendication 1, caractérisé en ce qu'on utilise un électrolyte solide de la famille des bêta-alumines.

3. Procédé selon la revendication 1, caractérisé en ce qu'on utilise, comme électrolyte solide, un supraconducteur ionique de sodium à base de sodium, de zirconium et de phosphate.

4. Procédé selon l'une quelconque des revendications précédentes, caractérisé en ce qu'on utilise l'aluminium comme métal liquide.

5. Procédé selon la revendication 4, caractérisé en ce que le sodium est l'autre élément chimique du groupe Ia.

6. Procédé selon l'une quelconque des revendications précédentes, caractérisé en ce qu'on utilise du bismuth ou un alliage de bismuth comme matière électroconductrice.
